

**United States Patent [19]**  
**Shibata**

[11] **Patent Number:** **4,479,892**  
[45] **Date of Patent:** **Oct. 30, 1984**

**[54] AG-METAL OXIDES ELECTRICAL  
CONTACT MATERIALS**

- [75] Inventor: Akira Shibata, Yokohama, Japan  
[73] Assignee: Chugai Denki Kogyo K.K., Japan  
[21] Appl. No.: 494,970  
[22] Filed: May 16, 1983  
[51] Int. Cl.<sup>3</sup> ..... H01B 1/02  
[52] U.S. Cl. ..... 252/514; 252/512;  
252/513  
[58] Field of Search ..... 252/514, 513, 512;  
419/50, 48, 64; 29/874, 875, 879

**[56] References Cited**

**U.S. PATENT DOCUMENTS**

- 3,859,087 1/1975 Backstrom ..... 252/513  
3,880,777 4/1975 Shibata ..... 252/519  
3,893,821 7/1975 Davies et al. ..... 252/514  
3,913,201 10/1975 Schreiner et al. ..... 252/521  
3,951,872 4/1976 Neely ..... 252/513  
3,957,453 5/1976 Hüssler et al. ..... 252/513

*Primary Examiner—Josephine L. Barr*

*Attorney, Agent, or Firm—Shlesinger, Fitzsimmons & Shlesinger*

**[57] ABSTRACT**

Electrical contact materials of a silver base which have dispersed in their silver matrices 2-20 weight % of either one of or combination of fine oxide grains of Sn, Sb, Zn, In, and Bi, and which materials are diffused at their contact surfaces and for moderate depths adjacent thereto with Au, Pd, or alloys thereof, which gradually diminish in diffusion density from the contact surfaces to the moderate depths of the contact materials. The precious metal thus diffused in solid phase about the contact surfaces prevents their chemical aging and improves electrical performance such as anti-weldability, contact resistance, and endurance, without scattering from the contact surfaces or melting deeply all together into the matrices of the contact materials, and further without isolating from and coagulating spherically on the contact surfaces, even when they are subjected to electric arcs.

**2 Claims, No Drawings**

## AG-METAL OXIDES ELECTRICAL CONTACT MATERIALS

### BACKGROUND OF THE INVENTION

In order to prevent the lowering of electrical performance of electrical contacts due to oxidation or sulfuration of silver or alloys thereof which form the contact surfaces of the electrical contacts, it has been suggested to have said contact surfaces plated or clad in a thickness of  $1\text{--}15\mu$  by gold, palladium, or alloys thereof which scarcely react with an environmental gas atmosphere. Such employment is effective for a certain extent when the electric density exerted on contact surfaces is comparatively low. However, when contacts are charged with electric current of a high density and they are exposed to arcs of a high temperature resulting from the opening and closing cycle of the contacts, gold, palladium, or alloys thereof which lie over the contact surfaces are scattered off from said surfaces or melt deeply all together into matrices of contacts, whereby the metals can not perform as well as desired.

Lately, it has been proposed and applied to have silver or silver alloy matrices dispersed with metal oxides such as Sn, Sb, Zn, In, and Bi oxides, so that contacts made therefrom can exhibit, on account of high refractoriness of the metal oxides, high anti-weldability and low-electric contact resistance, even when electric current of a high density is applied thereto. To our disappointment, however, employment of a precious metal of the kind mentioned above for plating or cladding surfaces of the just above-mentioned contacts exhibits little effect or brings forth adverse effects. To wit, since said silver-base contacts which are dispersed with refractory metal oxides are thermally highly stable, and hardly agitate even when their surfaces are subjected to arcs of a high temperature, which are frequently produced particularly at their initial stages of use, and since the more the contact surfaces are thus thermally stable, the more difficult it is to apply gold, palladium, or their alloys to such contact surfaces, because said precious metals are agitated one-sidedly when they are subjected to arcing heat, and they tend to be isolated from and coagulate spherically on the contact surfaces, resulting in the occurrence of undesirable welding of contacts and subsequent inability of making and breaking thereof.

### BRIEF SUMMARY OF THE INVENTION

In view of the above, one purpose of this invention is to provide a novel contact material of silver base which contains dispersedly in the silver matrix 2-20 weight % of one of, or a combination of, refractory and fine oxide grains of Sn, Sb, Zn, In, and Bi, and has a contact surface which is plated, coated by evaporation, or clad with a layer of gold, palladium, or their alloys of a thickness of  $2\text{--}5\mu$ , said precious metal having been diffused into the contact material in solid phase, viz., at a temperature below its melting point, preferably at a temperature of  $700\text{--}900^\circ\text{C}$ . and under pressure. Observation by E. D. M. of the electrical contact material made in accordance with this invention shows that the aforementioned precious metal occupies about 20-100 weight % of the contact material at its top surface area, and diffusely reaches to moderate or middle depths of the material, while reducing its density gradually. Thus, the precious metal which lies at the surface and has been diffused to the moderate depths of the contact, prevents

the contact surface from chemical aging such as sulfuration, oxidation, or chlorination thereof, and makes its contact surface stable. Said precious metal does not isolate from the contact surface even at the making and breaking operations with electric arcs. The contact material of this invention can advantageously be employed for the duty under a large electric current as well as under a low electric load, since its contact surface changes smoothly and evenly, with the progress of operation cycles, from a phase which is rich of the precious metal, to a phase where it is consisted of the precious metal, silver, and metal oxides, and then to a phase where it is consisted of silver and metal oxides. It shall be noted also that since the precious metal such as gold and alloys thereof which have diffused to silver matrices of the contact material, wet well with metal oxides which are dispersed in the matrices, the wettability of the metal oxides with silver is consequently improved, whereby the electric resistance of the contact material becomes more stable and its ductility which is of critical significance for shaping the material to a desired form is also improved.

It is of course possible that metal oxides of the kind mentioned above, can be replaced at least in part by Cd grain oxides. It is also possible of course that the contact material of this invention can contain and/or be clad opposite its contact surface with Ag, Cu, Ni, Fe, or their alloys.

### EXAMPLES

#### Example 1 (contact materials powder-metallurgically made by Ag-Sn (8 weight %))

##### Contact material (1-A)

92 weight % of Ag powder and 8 weight % of oxidized Sn powder, total weight of which is 3 kg., were mixed well in a shaking mill for 24 hours. This mixture was molded, by a rubber press of  $0.5\text{ T/cm}^2$ , to a billet of 50 mm in diameter and 130 mm in length. The billet was sintered in air at  $850^\circ\text{C}$ . for 2 hours. The billet which had been heated in advance to  $800^\circ\text{C}$ . was hot-rolled into a plate having a silver back of 0.1 mm in thickness. From the plate, square contacts of 0.5 mm (thickness including the silver back)  $\times 4\text{ mm} \times 4\text{ mm}$  were punched out.

##### Contact material (1-B)

The contacts of the above (1-A) were plated at contact surface thereof with  $6\mu$  of 20-karat gold.

##### Contact material (1-C)

The hot-rolled plate with the silver back of the above (1-A) was plated at its upper surface with  $3\mu$  of Au, and then hot-rolled at  $850^\circ\text{C}$ . From this plate, contacts of dimensions same to those of the above (1-A) were obtained. The observation by E. D. M. of the contacts showed that their top surfaces were almost all gold, and gold gradually reduced of its density and diffused to about  $4.5\mu$  in depth.

#### Example 2 (contact materials made by internal oxidation of Ag-Sn (7 weight %)-Bi (0.5 weight %) alloy)

##### Contact material (2-A)

A sheet of 0.5 mm in thickness of the alloy, Ag-Sn (7%) Bi (0.5%), with a silver back of 0.1 mm thickness was internally oxidized for 8 hours at an oxygen atmosphere of  $700^\circ\text{C}$ . of 8 atm. From this sheet, there were obtained contacts of dimensions same to those of the above (1-A).

## Contact material (2-B)

The contacts of the above (2-A) were plated at contact surfaces thereof with  $6\mu$  of 20-karat gold.

## Contact material (2-C)

The internally oxidized sheet of the above (2-A) was plated at its upper surface with  $2\mu$  of Au, and then hot-rolled at  $850^{\circ}$  C. in a hydrogen atmosphere into a thickness of 0.45 mm. There were obtained those square contacts of 0.45 mm (thickness including the silver back)  $\times$  4 mm  $\times$  4 mm in which gold was diffused on their upper surfaces and to middle depths.

Example 3 (contact materials made by internal oxidation of Ag-Sn (6 weight %)-In (3 weight %)-Ni (0.2 weight %) alloy

## Contact material (3-A)

Contacts were made by the steps same to the above (2-A).

## Contact material (3-B)

The contacts of the above (3-A) were plated at their contact surfaces with  $6\mu$  of 20-karat gold.

## Contact material (3-C)

By the employment of the above alloy, viz., Ag-Sn (6%)-In (3%)-Ni (0.2%), contacts were obtained by the steps same to the above (2-C).

Example 4 (contact materials made by internal oxidation of Ag-Cd (10 weight %)-Sn (2 weight %) alloy)

## Contact material (4-A)

Contacts were made by the steps same to the above (2-A).

## Contact material (4-B)

The contacts of the above (4-A) were plated at their contact surfaces with  $6\mu$  of 20-karat gold.

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1495

1500

1505

1510

1515

1520

1525

1530

1535

1540

contact materials, gradually reducing in density as the depth of diffusion increases, and occupying about 20-100 weight % of the contact surfaces of said materials.

2. Electrical contact materials as claimed in claim 1, 5

in which surfaces opposite to the contact surfaces are clad with Fe, Ag, Cu, Ni, or alloys thereof.

\* \* \* \* \*

10

15

20

25

30

35

40

45

50

55

60

65